# EUROPEAN PATENT SPECIFICATION

(11) **EP 2 128 233 B1**
(45) Date of publication and mention of the grant of the patent: **31.08.2016**
(21) Application number: 07859965.1
(22) Date of filing: 21.12.2007
(51) Int. Cl.: C10M 171/02, C10M 137/04, C10M 137/08, C10M 169/04, C10N 20/00, C10N 20/02, C10N 40/30

(54) **LUBRICANT COMPOSITION FOR ROTARY GAS COMPRESSOR AND USE IN A ROTARY GAS COMPRESSOR**
SCHMIERMITTELZUSAMMENSETZUNG FÜR ROTATIONSGASVERDICHTER UND VERWENDUNG IN EINEM ROTATIONSGASVERDICHTER
COMPOSITION LUBRIFIANTE POUR COMPRESSEUR À GAZ ROTATIF ET L'UTILISATION DANS UN COMPRESSEUR À GAZ TOURNANT

(30) Priority: 23.01.2007 JP 2007013084
(43) Date of publication of application: 02.12.2009
(73) Proprietor: Idemitsu Kosan Co., Ltd., Chiyoda-ku Tokyo 100-8321 (JP)
(72) Inventor: KAMIMURA, Hideto, Ichihara-shi Chiba 299-0107 (JP)
(74) Representative: Hoffmann Eitle
(86) International application number: PCT/JP2007/074685
(87) International publication number: WO 2008/090706

(56) References cited:
- WO-A1-98/58042
- WO-A1-2006/120925
- WO-A2-2006/122979
- JP-A- 07 126 673
- JP-A- 2005 154 760
- JP-A- 2005 155 461
- JP-A- 2005 213 447
- DATABASE WPI Week 200545 Thomson Scientific, London, GB; AN 2005-438982 XP002629614, & JP 2005 154760 A (IDEMITSU KOSAN CO LTD) 16 June 2005 (2005-06-16)

## Description

### Technical Field

The present invention relates to a lubricating oil composition for a rotary gas compressor and the use of the same in a rotary gas compressor.

### Background Art

A rotary gas compressor, which generates less vibration than a reciprocating gas compressor, is operated with a massive amount of a lubricating oil being injected, so that a temperature of discharged gas can be lowered. Among the rotary gas compressor, an oil-cooling screw compressor, which is a positive displacement type, has features of a rotary type as well as features of the positive displacement type. Owing to the features such as high efficiency, compact size and long-period continuous operation, the oil-cooling screw compressor has been widely used in the industry (for example, Patent Documents 1 and 2). A lubricating oil having a high kinematic viscosity of more than 5 mm²/s at 100 degrees C is typically used for such compressor.

Patent Document 1: JP-A-09-151870
Patent Document 2: JP-A-11-013661

### Disclosure of the Invention

### Problems to Be Solved by the Invention

Since such a typical rotary gas compressor (oil-cooling screw compressor) as disclosed in Patent Documents 1 and 2 has used the lubricating oil of high viscosity as described above, a driving power becomes excessive when the rotary gas compressor is operated. Resultantly, a sufficient performance for energy-saving has not been obtainable. WO 2006/122979 A2 relates to the use of a Fischer-Tropsch derived white oil in food contact applications. One example of this white oil has a flash point of 232°C, a kinemetic viscosity at 100°C of 4.3 mm²/s and a boiling point at 5% distillation of 409°C.
JP 2005/154760 pertains to a lubricant base oil having a high viscosity index and a low temperature fluidity, and a lubricating oil composition which is excellent in a high viscosity index, high shear stability and high oxidation stability with a high flash point and a low density. This document seems to describe one base oil having a flash point of 238°C, a kinemetic viscosity at 100°C of 4.847 mm²/s and a boiling point at 5% distillation of 386°C. It also seems to describe one lubricating oil composition having a kinemetic viscosity at 100°C of 4.263 mm²/s.
WO 2006/120925 A1 relates to a process for producing saturated aliphatic hydrocarbon compounds and a lubricant composition containing the same. Table 2 of this document relates to a lubricant composition having a kinemetic viscosity at 100°C of 7.15 mm²/s.

Accordingly, an object of the invention is to provide a lubricating oil composition for a rotary gas compressor and the use of the same in a rotary gas compressor, the lubricating oil composition having a sufficient lubricity performance as well as excellent capability of energy-saving and reducing a lubricating oil consumption.

### Means for Solving the Problems

As a result of a dedicated studies for solving the problem, the inventors have found that a lubricating oil composition is particularly excellently applicable to a rotary gas compressor when a kinematic viscosity, a flash point and a distillation temperature of the lubricating oil composition are within a particular range, and then the invention have been achieved.

The invention provides a lubricating oil composition for a rotary gas compressor and the use of the same in a rotary gas compressor as described below:
(1) A lubricating oil composition for a rotary gas compressor, wherein said lubricating oil composition contains a lubricating base oil having a kinematic viscosity at 40 degrees C from 10 to 68 mm²/s, and a phosphorus compound antioxidant, the phosphorus compound antioxidant being contained in an amount from 0.01 mass% to 10 mass% based on the total amount of the composition, the composition having a kinematic viscosity of 5 mm²/s or less at 100 degrees C; a flash point according to JIS K 2265 of 200 degrees C or more; and a 5 volume % distillation temperature according to JIS K 2254 of 350 degrees C or more.
(2) The lubricating oil composition for a rotary gas compressor as described in (1), wherein a kinematic viscosity at 40 degrees C is 28 mm²/s or less.
(3) The lubricating oil composition for a rotary gas compressor as described in (1) or (2), wherein the phosphorus compound antioxidant is contained in an amount from 0.03 mass% to 5 mass% based on the total amount of the composition.
(4) The lubricating oil composition for a rotary gas compressor as described in any one of (1) to (3), wherein the 5 volume % distillation temperature is 390 degree C or more.
(5) The lubricating oil composition for a rotary gas compressor as described in any one of (1) to (4), wherein the lubricating base oil is selected from API (American Petroleum Institute) classification group II.
(6) The lubricating oil composition for a rotary gas compressor as described in any one of (1) to (5), further comprising a phosphorus extreme pressure agent.
(7) The lubricating oil composition for a rotary gas compressor as described in any one of (1) to (6), wherein the phosphorus extreme pressure agent is contained in an amount from 0.01 mass% to 10 mass% based on the total amount of the composition.
(8) Use of the lubricating oil composition for a rotary gas compressor as described in any one of (1) to (7) in a rotary compressor.

When the lubricating oil composition for the rotary gas compressor according to the above aspect of the invention is filled in the rotary gas compressor and the rotary gas compressor is operated, a sufficient lubricity performance is maintainable, while an energy-saving effect is excellent owing to a low kinematic viscosity. Further, owing to a low evaporativity of the lubricating oil composition, an evaporation loss is small even when the rotary gas compressor is operated for long hours. The lubricating oil composition for the rotary gas compressor according to the above aspect of the invention is considerably effective particularly when being filled in an oil-cooling crew compressor.

### Best Mode for Carrying Out the Invention

Embodiments of the invention will be described in detail below. A lubricating oil composition for a rotary gas compressor according to an aspect of the invention (referred to as "the composition" hereinafter) contains a lubricating base oil having a kinematic viscosity at 40 degrees C from 10 to 68 mm²/s, and an amine compound antioxidant and a phosphorus compound antioxidant, the amine compound antioxidant and the phosphorus compound antioxidant being contained in an amount from 0.01 mass% to 10 mass% based on the total amount of the composition, the composition having a kinematic viscosity of 5 mm²/s or less at 100 degrees C; a flash point according to JIS K 2265 of 200 degrees C or more; and a 5 volume % distillation temperature according to JIS K 2254 of 350 degrees C or more.

The lubricant base oil is not particularly limitative, but any oil typically used as a lubricant base oil can be used irrespective of a mineral oil or a synthetic oil.

Preferably, examples of the mineral oil may include paraffinic and naphthenic base oils which can be obtained by subjecting a lubricating oil fraction produced by atmospheric- and vacuum-distillation of a crude oil, to any suitable combination of refining processes selected from solvent-deasphalting, solvent-extracting, hydrocracking, solvent-dewaxing, catalytic-dewaxing, hydrorefining, sulfuric acid treatment and clay treatment.

Preferably, examples of the synthetic oil may include: a poly-α-olefin (1-octene oligomer, 1-decene oligomer and the like), a polybutene, an isoparaffin, an olefin copolymer (an ethylene-propylene copolymer and the like), an alkylbenzene, an alkyl naphthalene, monoester (butyl stearate and the like), a dibasic acid ester (ditridecyl glutarate, di-2-ethylhexyladipate, diisodecyladipate, ditridecyladipate, di-2-ethylhexlsebacate and the like), a tribasic acid ester (tri-merit acid ester and the like), a polyol ester (trimethylol propane caplyrate, trimethylol propane pelargonate, pentaerythritol 2-ethylhexanoate, pentaerythritol pelargonate, and the like), a polyoxyalkylene glycol, a dialkyl diphenyl ether, an alkyl diphenyl sulfide, a polyphenyl ether, silicone oil (dimethyl silicone and the like) and a perfluoropolyether.

These mineral oils and synthetic oils may be singularly used, or two or more base oils selected from these oils may be mixed at any rate in use.

The base oil of any viscosity may be used for the composition. However, in consideration of lubricity, cooling performance and friction loss at agitation, it is desirable to use the base oil with a kinematic viscosity of 1 to 10,000 mm²/s at 40 degrees C, preferably 5 to 100 mm²/s, more preferably 10 to 68 mm²/s. The base oil for the composition may be preferably selected from API (American Petroleum Institute) classification groups II to IV.

It is preferable that the lubricating oil composition for the rotary gas compressor according to the aspect of the invention contains a phosphorous extreme pressure agent.

The phosphorous extreme pressure agent is preferably orthophosphoric esters, phosphite esters, acidic phosphate esters, acidic phosphite esters or an amine salt thereof.

The orthophosphoric ester may be exemplified by a triaryl phosphate, a trialkyl phosphate, a trialkyl aryl phosphate, a triaryl alkyl phosphate and a trialkenyl phosphate, examples of which may include: a triphenyl phosphate, a tricresyl phosphate, a benzyl diphenyl phosphate, an ethyl diphenyl phosphate, a tributyl phosphate, an ethyl dibutyl phosphate, a cresyl diphenyl phosphate, a dicresyl phenyl phosphate, an ethylphenyl diphenyl phosphate, a diethylphenyl phenyl phosphate, a propylphenyl diphenyl phosphate, a dipropylphenyl phenyl phosphate, a triethylphenyl phosphate, a tripropylphenyl phosphate, a butylphenyl diphenyl phosphate, a dibutylphenyl phenyl phosphate, a tributylphenyl phosphate, a trihexyl phosphate, a trinormal octyl phosphate, a tri(2-ethylhexyl) phosphate, a tridecyl phosphate, a trilauryl phosphate, a trimyristyl phosphate, a tripalmityl phosphate, a tristearyl phosphate, a trioleyl phosphate and the like.

Examples of the phosphite ester may include: a triethyl phosphite, a tributyl phosphite, a triphenyl phosphite, a tricresyl phosphite, a tri(nonylphenyl)phosphite, a tri(2-ethylhexyl)phosphite, a tridecyl phosphite, a trilauryl phosphite , a triisooctyl phosphite, a diphenylisodecyl phosphite, a tristearyl phosphite, a trioleyl phosphite and the like.

Examples of the acidic phosphate ester may include: a 2-ethylhexyl acid phosphate, a dinormal octyl acid phosphate, an ethyl acid phosphate, a butyl acid phosphate, an oleyl acid phosphate, a tetracosyl acid phosphate, an isodecyl acid phosphate, a lauryl acid phosphate, a tridecyl acid phosphate, a stearyl acid phosphate, an isostearyl acid phosphate and the like.

Examples of the acidic phosphite ester may include: a diethyl hydrogen phosphite, a dibutyl hydrogen phosphite, a dilauryl hydrogen phosphite, a dioleyl hydrogen phosphite, a distearyl hydrogen phosphite, a diphenyl hydrogen phosphite and the like. Examples of amines to form the amine salt of the above compounds may include: a mono-substituted amine, a di-substituted amine or a tri-substituted amine represented by the following formula (1). The alkyl group or the alkenyl group having 3 to 30 carbon atoms represented by R in the formula (1) may be linear, branched or cyclic.

RnNH3-n (1)

In the formula: R represents an alkyl group or an alkenyl group having 3 to 30 carbon atoms, preferably 4 to 18 carbon atoms, an aryl group or an arylalkyl group having 6 to 30 carbon atoms, preferably 6 to 15 carbon atoms, or a hydroxyalkyl group having 2 to 30 carbon atoms, preferably 2 to 18 carbon atoms; and n represents 1, 2 or 3. When plural units of R are contained, the plural units of R may be mutually the same or different.

Examples of the mono-substituted amine may include: a butyl amine, a pentyl amine, a hexyl amine, a cyclohexyl amine, an octyl amine, a lauryl amine, a stearyl amine, an oleyl amine, a benzyl amine and the like. Examples of the di-substituted amine may include: a dibutyl amine, a dipentyl amine, a dihexyl amine, a dicyclohexyl amine, a dioctyl amine, a dilauryl amine, a distearyl amine, an dioleyl amine, a dibenzyl amine, a stearyl monoethanol amine, a decyl monoethanol amine, a hexyl monopropanol amine, a benzyl monoethanol amine, a phenyl monoethanol amine, tolyl monopropanol and the like. Examples of the tri-substituted amine may include: a tributyl amine, a tripentyl amine, a trihexyl amine, a tricyclohexyl amine, a trioctyl amine, a trilauryl amine, a tristearyl amine, a trioleyl amine, a tribenzyl amine, a dioleyl monoethanol amine, a dilauryl monopropanol amine, a dioctyl monoethanol amine, a dihexyl monopropanol amine, a dibutyl monopropanol amine, an oleyl diethanol amine, a stearyl dipropanol amine, a lauryl diethanol amine, an octyl dipropanol amine, a butyl diethanol amine, a benzyl diethanol amine, a phenyl diethanol amine, a tolyl dipropanol amine, a xylyl diethanol amine, a triethanol amine, a tripropanol amine, a tertiary dodecyl amine and the like.

Among the phosphorous extreme pressure agents, tricresyl phosphate and a diethyl hydrogen phosphite tertiary dodecyl amine salt are preferable in perspective of heat resistance.

In view of blending effects and an economical aspect, a content of the extreme pressure agent is typically approximately 0.01 to 30 mass% of the total amount of the lubricating oil composition, preferably 0.01 to 10 mass%.

The lubricating oil composition of the present invention contains a phosphorus compound antioxidant. Examples of the amine compound may include: a monoalkyldiphenylamine compound such as monooctyldiphenylamine and monononyldiphenylamine; a dialkyl diphenylamine compound such as 4,4'-dibutyldiphenylamine, 4,4'-dipentyldiphenylamine, 4,4'-dihexyldiphenylamine, 4,4'-diheptyldiphenylamine, 4,4'-dioctyldiphenylamine and 4,4'-dinonyldiphenylamine; a polyalkyldiphenylamine compound such as tetrabutyldiphenylamine, tetrahexyldiphenylamine, tetraoctyldiphenylamine and tetranonyldiphenylamine; and a naphthylamine compound such as α-naphthylamine, phenyl-α-naphthylamine, butylphenyl-α-naphthylamine, pentylphenyl-α-naphthylamine, hexylphenyl-α-naphthylamine, heptylphenyl-α-naphthylamine, octylphenyl-α-naphthylamine, nonylphenyl-α-naphthylamine, decylphenyl-α-naphthylamine, dodecylphenyl-α-naphthylamine and the like.

Examples of the phosphorous compound, may include: the phosphorous compound such as diethyl[[3,5-bis(1,1-dimethylethyl)-4-hydroxyphenyl]methyl]phosphonate, zinc dialkyldithiophosphate such as zinc di-2-ethylhexyldithiophosphate and a thioterpene compound such as a reactant of phosphorous pentasulfide and pinene.

Among the antioxidants, diethyl[[3,5-bis(1,1-dimethylethyl)-4-hydroxyphenyl]methyl]phosphonate is preferable in perspective of heat resistance.

A content of the antioxidant is approximately 0.01 to 10 mass% of the total amount of the lubricating oil composition, preferably 0.03 to 5 mass%.

The composition, which is preferably formed of the above-described base oil and various additives, has a kinematic viscosity (according to JIS (Japanese Industrial Standard) K 2283) of 5 mm²/s or less at 100 degrees C, preferably 4.95 mm²/s or less, more preferably 4.5 mm²/s or less. When the kinematic viscosity at 100 degrees C exceeds 5 mm²/s, the driving power of the rotary gas compressor is excessive.

A flash point of the composition (according to C.O.C, JIS K 2265) is 200 degrees C or more, preferably 210 degrees C or more, more preferably 220 degrees C or more. When the flash point is less than 200 degrees C, there is an increasing danger of flashing in operation of the rotary gas compressor filled with the composition.

5 volume % distillation temperature of the composition (according to JIS K 2254) is 350 degrees C or more, preferably 370 degrees C or more, more preferably 390 degrees C or more. In case where 5 volume % distillation temperature is less than 350 degrees C, lubricating oil consumption unpreferably increases when the rotary gas compressor is operated for long hours.

The rotary gas compressor filled with the above composition as a lubricating oil consumes less the lubricating oil and maintains a sufficient lubricity, thereby exhibiting an excellent energy-saving effect. Particularly, when the composition is filled in an oil-cooling screw compressor, the composition exhibits considerably excellent cooling performance and heat resistance.

The kinematic viscosity of the composition at 40 degrees C is preferably 28 mm²/s or less, more preferably 25 mm²/s or less, more preferably 23 mm²/s or less. When the kinematic viscosity at 40 degrees C exceeds 28 mm²/s, the driving power of the rotary gas compressor is excessive.

The lubricating oil composition for the rotary gas compressor according to the aspect of the invention may be further added with an oiliness agent, a rust inhibitor, a detergent dispersant, a metal deactivator and an antifoaming agent as needed.

The oiliness agent may be exemplified by an aliphatic alcohol, a fatty acid compound such as a fatty acid and a fatty acid metal salt, an ester compound such as a polyol ester, a sorbitan ester and a glyceride and an amine compound such as an aliphatic amine. The ester compound is preferable among these compounds since the ester compound can provide both heat resistance and lubricity.

In view of blending effects, a content of the oiliness agent is typically approximately 0.1 to 30 mass% of the total amount of the lubricating oil composition, preferably 0.5 to 10 mass%.

The rust inhibitor may be exemplified by a metal sulfonate, aliphatic amines, an organic phosphite ester, an organic phosphate ester, an organic metal sulfonate, an organic metal phosphate, an alkenyl succinic acid ester, a multivalent alcohol ester and the like. In view of blending effects, a content of the rust inhibitor is typically approximately 0.01 to 10 mass% of the total amount of the lubricating oil composition, preferably 0.05 to 5 mass%.

The detergent dispersant may be exemplified by a metal sulfonate, a metal salicylate, a metal phenate, a metal phosphonate and succinimide. A metallic detergent dispersant is preferable among these in perspective of detergent dispersivity and demulsification performance.

In view of blending effects, a content of the detergent dispersant is typically approximately 0.1 to 30 mass% of the total amount of the lubricating oil composition, preferably 0.5 to 10 mass%.

The metal deactivator may be exemplified by benzotriazoles and thiadiazoles. In view of blending effects, a content of the metal deactivator is typically approximately 0.01 to 10 mass% of the total amount of the lubricating oil composition, preferably 0.01 to 1 mass%.

The antifoaming agent may be exemplified by methyl silicone oil, fluorosilicone oil and polyacrylates. In view of blending effects, a content of the antifoaming agent is typically approximately 0.0005 to 0.01 mass% of the total amount of the lubricating oil composition.

### Examples

The invention will be further described in detail below with reference to Examples and Comparatives, which by no means limit scope of the invention.

### [Examples 1 to 6 and Comparatives 1 and 2]

Additives were added to predetermined base oils (API classification groups I to IV) to prepare lubricating oil compositions having respective properties. Maximum loading capacity, wear resistance, evaporation amounts and actual power consumption were evaluated. A method of examining properties of the lubricating oil compositions and a method for evaluating respective properties are shown below. Results are shown in Table 1.

### (1) Properties of Lubricating Oil Composition

A method of examining each property (standard) is shown below.
(1.1) Kinematic Viscosity (100 degrees C, 40 degrees C): according to JIS K 2283
(1.2) Viscosity Index: according to JIS K 2283
(1.3) Density (at 15 degrees C): according to JIS K 2249
(1.4) Flash Point (C.O.C): according to JIS K 2265
(1.5) Distillation Property (5 volume % distillation temperature, 10 volume % distillation temperature): according to JIS K 2254 (Distillation was conducted at reduced pressure of 133MPa and an obtained value was converted to a value at atmospheric pressure.)

### (2) Evaluation Items and Evaluation Method

### (2.1) Maximum Loading Capacity Test (Shell EP Test)

A test was conducted at a rotational speed of 1,800 rpm and at room temperature according to ASTM D2783. A load wear index (LWI) was obtained from a last non-seisure load (LNL) and a weld load (WL). The larger this value is, the better a load resistance is.

### (2.2) Wear Resistance Test (Shell Wear Test)

A test was conducted under conditions of a load of 392N, a rotational speed of 1,200 rpm, an oil temperature of 80 degrees C and a testing time of 60 minutes according to ASTM D2783. An average wear track diameter was calculated by averaging wear track diameters of three half-inch balls.

### (2.3) Film Residue Test

In a vessel based on JIS K 2540, a sample of 1g was filled. Air was flowed into the vessel under an atmosphere at a constant temperature of 150 degrees C with a flowing volume of 10 L/h for 6 hours. After the test, a mass of the sample (evaporation residue) was measured. An amount of the evaporation residue relative to the original amount of the sample was expressed by mass percentage.

### (2.4) Actual Power Consumption

A commercially available oil-cooling screw compressor (motor output: 22kW, oil quantity: 10L, intake gas: air, intake pressure: atmospheric pressure, intake temperature: 25 degrees C) was used as a rotary gas compressor to measure effective power consumption of the compressor motor when continuously operated for three hours at an average oil temperature of 80 degrees C. The measurement was conducted by a clamp-on-sensor type power meter that is commercially available.

The measurement was conducted in two operation modes as follows.
Operation Mode I: discharge pressure of 0.65 MPa
Operation Mode II: discharge pressure of 0.24 MPa

**[Table 1]**

| | | Example 1 | Example 2 | Example 3 | Example 4 | Example 5 | Example 6 | Comparative 1 | Comparative 2 |
|---|---|---|---|---|---|---|---|---|---|
| base oil (mass%) | API GII (100 neutral) | remnant | | | remnant | remnant | remnant | | |
| | API GIII (100 neutral) | | remnant | | | | | | |
| | API GIV (100 neutral) | | | remnant | | | | | |
| | API GII (150 neutral) | | | | | | 65 | remnant | |
| | API GI (100 neutral) | | | | | | | | remnant |
| additives (mass%) | dioctyldiphenylamine | 2 | 2 | 2 | 2 | 2 | 2 | 2 | 2 |
| | octylphenyl-α-naphthylamine | 1 | 1 | 1 | 1 | 1 | 1 | 1 | 1 |
| | phosphorous containing antioxidant *1 | 0.5 | 0.5 | 0.5 | 0.5 | 0.5 | 0.5 | 0.5 | 0.5 |
| | ester oiliness agent *2 | - | - | - | - | 10 | - | - | - |
| | tricresyl phosphate | - | - | - | 0.4 | - | - | - | - |
| | amine salt of phosphate ester | - | - | - | 0.02 | - | - | - | - |
| | other additives *3 | 0.2 | 0.2 | 0.2 | 0.2 | 0.2 | 0.2 | 0.2 | 0.2 |
| properties | kinematic viscosity (100 °C)(mm²/s) | 4.284 | 4.230 | 3.900 | 4.291 | 4.300 | 4.931 | 5.346 | 4.208 |
| | kinematic viscosity (40 °C)(mm²/s) | 20.44 | 19.57 | 17.50 | 20.51 | 20.30 | 26.58 | 30.98 | 20.54 |
| | viscosity index | 116 | 122 | 120 | 116 | 120 | 110 | 105 | 108 |
| | density (15°C)(g/cm³) | 0.8428 | 0.8338 | 0.8190 | 0.8431 | 0.8482 | 0.8558 | 0.8630 | 0.8577 |
| | flash point (COC)(°C) | 212 | 230 | 222 | 212 | 215 | 218 | 222 | 210 |
| | distillation property - 5 volume % distillation temperature (°C) | 375 | 398 | 417 | 376 | 377 | 375 | 374 | 346 |
| | distillation property - 10 volume % distillation temperature (° C) | 388 | 406 | 422 | 388 | 390 | 390 | 393 | 351 |
| evaluation | Shell EP LWI (N) | 165 | 171 | 164 | 301 | 307 | 163 | 164 | 170 |
| | Shell wear (mm) | 0.58 | 0.59 | 0.56 | 0.31 | 0.33 | 0.59 | 0.57 | 0.55 |
| | film residue (mass%) | 89.9 | 92.0 | 95.5 | 90.2 | 93.4 | 88.6 | 87.1 | 75.5 |
| | actual power consumption - operation mode I (kWh) | 67.731 | 67.647 | 67.136 | 67.741 | 67.756 | 68.730 | 69.280 | 67.613 |
| | actual power consumption - operation mode II (kWh) | 28.320 | 28.255 | 27.820 | 28.330 | 28.341 | 29.161 | 29.631 | 28.225 |

| | | | | | | | | | |
|---|---|---|---|---|---|---|---|---|---|
| *1 diethyl[[3,5-bis(1,1-dimethylethyl)-4-hydroxyphenyl]methyl]phosphonate *2 trimethylol propane trialkyl ester (in which an alkyl group is a mixture of C8 and C10) *3 a package of a metallic detergent dispersant, metallic rust inhibitor and antifoaming agent | | | | | | | | | |

### [Evaluation Results]

As shown in Table 1, the results of Examples 1 to 6 using the composition exhibited excellent lubricity performance as a lubricating oil as well as excellent energy-saving effect and consumed less lubricating oil. In contrast, in Comparative 1, a kinematic viscosity at 100 degrees C is high and power consumption of a rotary gas compressor is large. Moreover, a consumption of a lubricating oil is rather large irrespective of the high kinematic viscosity at 100 degrees C. In Comparative 2, a consumption of a lubricating oil becomes excessive due to a low 5 volume % distillation temperature, thereby making it difficult to operate a rotary gas compressor for long hours.

### Industrial Applicability

The present invention is preferably applicable as a lubricating oil for a rotary gas compressor.

## Claims

1. A lubricating oil composition for a rotary gas compressor, wherein said lubricating oil composition contains
a lubricating base oil having a kinematic viscosity at 40 degrees C from 10 to 68 mm²/s, and a phosphorus compound antioxidant, the phosphorus compound antioxidant being contained in an amount from 0.01 mass% to 10 mass% based on the total amount of the composition,
the composition having:
a kinematic viscosity of 5 mm²/s or less at 100 degrees C; a flash point according to JIS K 2265 of 200 degrees C or more; and a 5 volume % distillation temperature according to JIS K 2254 of 350 degrees C or more.

2. The lubricating oil composition for a rotary gas compressor according to claim 1, wherein
a kinematic viscosity at 40 degrees C is 28 mm²/s or less.

3. The lubricating oil composition for a rotary gas compressor according to any one of claims 1 to 2, wherein
the phosphorus compound antioxidant is contained in an amount from 0.03 mass% to 5 mass% based on the total amount of the composition.

4. The lubricating oil composition for a rotary gas compressor according to any one of claims 1 to 3, wherein the 5 volume % distillation temperature is 390 degree C or more.

5. The lubricating oil composition for a rotary gas compressor according to any one of claims 1 to 4, wherein the lubricating base oil is selected from API (American Petroleum Institute) classification group II.

6. The lubricating oil composition for a rotary gas compressor according to any one of claims 1 to 5, further comprising a phosphorus extreme pressure agent.

7. The lubricating oil composition for a rotary gas compressor according to claim 6, wherein the phosphorus extreme pressure agent is contained in an amount from 0.01 mass% to 10 mass% based on the total amount of the composition.

8. Use of the lubricating oil composition for a rotary gas compressor according to any one of claims 1 to 7 in a rotary compressor.

## Patentansprüche

1. Schmiermittelölzusammensetzung für einen Rotationsgaskompressor, worin die Schmiermittelölzusammensetzung enthält:
ein Schmiermittel-Basisöl mit einer kinematischen Viskosität bei 40°C von 10 bis 68 mm²/s und ein Antioxidans aus einer Phosphorverbindung, wobei das Antioxidans aus der Phosphorverbindung in einer Menge von 0,01 bis 10 Massen-%, bezogen auf die Gesamtmenge der Zusammensetzung, enthalten ist,
wobei die Zusammensetzung hat:
eine kinematische Viskosität von 5 mm²/s oder weniger bei 100°C, einen Flashpunkt gemäß JIS K 2265 von 200°C oder mehr und eine 5 Vol.-%-ige Destillationstemperatur gemäß JIS K 2254 von 350°C oder mehr.

2. Schmiermittelölzusammensetzung für einen Rotationsgaskompressor nach Anspruch 1, worin eine kinematische Viskosität bei 40°C 28 mm²/s oder weniger ist.

3. Schmiermittelölzusammensetzung für einen Rotationsgaskompressor nach einem der Ansprüche 1 bis 2, worin das Antioxidans aus der Phosphorverbindung in einer Menge von 0,03 bis 5 Massen-% enthalten ist, bezogen auf die Gesamtmenge der Zusammensetzung.

4. Schmiermittelölzusammensetzung für einen Rotationsgaskompressor nach einem der Ansprüche 1 bis 3, worin die 5 Vol.-%-ige Destillationstemperatur 390°C oder mehr ist.

5. Schmiermittelölzusammensetzung für einen Rotationsgaskompressor nach einem der Ansprüche 1 bis 4, worin das Schmiermittelbasisöl ausgewählt ist aus der API (American Petroleum Institute)-Klassifizierungsgruppe II.

6. Schmiermittelölzusammensetzung für einen Rotationsgaskompressor nach einem der Ansprüche 1 bis 5, weiterhin umfassend ein phosphorhaltiges extremes Druckmittel.

7. Schmiermittelölzusammensetzung für einen Rotationsgaskompressor nach Anspruch 6, worin das phosphorhaltige extreme Druckmittel in einer Menge von 0,01 bis 10 Massen-% enthalten ist, bezogen auf die Gesamtmenge der Zusammensetzung.

8. Verwendung der Schmiermittelölzusammensetzung für einen Rotationsgaskompressor gemäß einem der Ansprüche 1 bis 7 in einem Rotationskompressor.

## Revendications

1. Composition d'huile lubrifiante pour un compresseur à gaz rotatif, dans laquelle ladite composition d'huile lubrifiante contient
une huile lubrifiante de base ayant une viscosité cinématique à 40 °C de 10 à 68 mm²/s, et un antioxydant à base d'un composé de phosphore, l'antioxydant à base d'un composé de phosphore étant contenu en une quantité de 0,01 % en masse à 10 % en masse, par rapport à la quantité totale de la composition,
la composition ayant :
une viscosité cinématique de 5 mm²/s ou moins à 100 °C ; un point d'éclair selon JIS K 2265 de 200 °C ou plus ; et une température de distillation de 5 % en volume selon JIS K 2254 de 350 °C ou plus.

2. Composition d'huile lubrifiante pour un compresseur à gaz rotatif selon la revendication 1, dans laquelle une viscosité cinématique à 40 °C est de 28 mm²/s ou moins.

3. Composition d'huile lubrifiante pour un compresseur à gaz rotatif selon l'une quelconque des revendications 1 à 2, dans laquelle
l'antioxydant à base d'un composé de phosphore est contenu en une quantité de 0,03 % en masse à 5 % en masse, par rapport à la quantité totale de la composition.

4. Composition d'huile lubrifiante pour un compresseur à gaz rotatif selon l'une quelconque des revendications 1 à 3, dans laquelle la température de distillation de 5 % en volume est de 390 °C ou plus.

5. Composition d'huile lubrifiante pour un compresseur à gaz rotatif selon l'une quelconque des revendications 1 à 4, dans laquelle l'huile lubrifiante de base est choisie dans le groupe II de la classification API (American Petroleum Institute).

6. Composition d'huile lubrifiante pour un compresseur à gaz rotatif selon l'une quelconque des revendications 1 à 5, comprenant en outre un agent de pression extrême à base de phosphore.

7. Composition d'huile lubrifiante pour un compresseur à gaz rotatif selon la revendication 6, dans laquelle l'agent de pression extrême à base de phosphore est contenu en une quantité de 0,01 % en masse à 10 % en masse, par rapport à la quantité totale de la composition.

8. Utilisation de la composition d'huile lubrifiante pour un compresseur à gaz rotatif selon l'une quelconque des revendications 1 à 7 dans un compresseur rotatif.
